# EUROPEAN PATENT SPECIFICATION

(11) **EP 3 293 278 B1**
(45) Date of publication and mention of the grant of the patent: **09.03.2022**
(21) Application number: 17020405.1
(22) Date of filing: 06.09.2017
(51) Int. Cl.: C22C 21/00, C22C 21/02, C22C 21/06, C22C 21/04, B22D 21/00, B22D 17/00

(54) **HYPEREUTECTIC HIGH PRESSURE DIE CAST ALUMINUM-SILICON CAST ALLOY**
HYPEREUTEKTISCHE ALUMINIUM SILICIUM HOCHDRUCKGUSSLEGIERUNG
ALLIAGE HYPEREUTECTIQUE ALUMINIUM SILICIUM POUR COULEE SOUS HAUTE PRESSION

(30) Priority: 13.09.2016 US 201615263859
(43) Date of publication of application: 14.03.2018
(73) Proprietor: Brunswick Corporation, Mettawa, IL 60045 (US)
(72) Inventor: Donahue, Raymond J., Fond du Lac, WI 54937 (US); Anderson, Kevin R., Fond du Lac, WI 54935 (US); Cleary, Terrance M., Fond du Lac, WI 54935 (US); Monroe, Alexander K., St. Cloud, WI 53079 (US)
(74) Representative: Von Rohr Patentanwälte Partnerschaft mbB

(56) References cited:
- US-B1- 6 168 675
- US-B2- 7 666 353
- DAVAMI P ET AL: "Strontium as a modifying agent for Al-Si eutectic alloy", BRITISH FOUNDRY, INSTITUTE OF BRITISH FOUNDRYMEN, CHESTERFIELD, GB, vol. 72, no. 4, 1 January 1979 (1979-01-01), pages 4-7, XP009064981, ISSN: 0007-0718
- DINNIS C M ET AL: "The influence of strontium on porosity formation in Al-Si alloys", METALLURGICAL AND MATERIALS TRANSACTIONS A: PHYSICAL METALLURGY & MATERIALS SCIE, ASM INTERNATIONAL, MATERIALS PARK, OH, US, vol. 35A, no. 11, 1 November 2004 (2004-11-01), pages 3531-3541, XP009064933, ISSN: 1073-5623, DOI: 10.1007/S11661-004-0190-9
- Barrie S Shabel ET AL: "Friction and Wear of Aluminum-Silicon Alloys" In: 1 January 1992 (1992-01-01), ASM International, XP55447945, vol. 18, pages 785-794, DOI: 10.1361/asmhba0002331, * paragraph [Metallurgy.of.Al/Si.ALLOYS] * * tables 1,5 * * paragraphs [00Al] - [Si.ALLOYS.Applications] *

## Description

The present invention relates to a hypereutectic high pressure die cast aluminum silicon alloy.

The eutectic structure of aluminum silicon alloys has long been studied to determine the mechanical properties of the alloys, see US 1,387,900 A and US 1,410,461 A. After more than 80 years of studying this eutectic structure, those skilled in the art now understand that sodium or strontium additions to the eutectic melt in only 100 ppm concentrations changes the size and morphology of the eutectic silicon phase resulting in a significant increase in the alloy's ductility.

Still, hypereutectic aluminum silicon alloys are not used to a great extent in sand casting processes because they are difficult to machine and because the primary silicon particle size is larger at sand casting cooling rates than at cooling rates for casting processes that use metal molds. As a result, there is a requirement to control the casting's microstructure in order to achieve an acceptable machinability. Achieving an acceptable machinability in a hypereutectic alloy is typically accomplished through phosphorus additions to the alloy melt to refine the primary silicon particle size. However, phosphorus prefers to form phosphides with common melt additives such as strontium and sodium rather than reacting with aluminum to form aluminum phosphide. This is problematic because aluminum phosphide is the nucleus for primary silicon formation in the eutectic structure of hypereutectic aluminum silicon alloys. Accordingly, the eutectic structure of phosphorus containing hypereutectic aluminum silicon alloys is always unmodified.

Thus, phosphorus refined, solution heat treated, quenched and aged, hypereutectic aluminum silicon structures provide the baseline for machinability, yet this baseline generally requires diamond tooling for proper machining. In contrast, eutectic aluminum silicon alloys and hypoeutectic aluminum silicon alloys, where the eutectic silicon structure is modified with strontium or sodium additions, have increased ductilities and are easier to machine. However, when the modified eutectic in the hypoeutectic alloy structures are compared to unmodified structures, the strontium or sodium modified eutectic structures exhibit nearly identical machinability in the heat treated condition with the unmodified structures. It is believed that this equivalence in machinability is due to the eutectic silicon phase occurring as a continuous phase in the eutectic whether the eutectic is modified or unmodified. Further, since it is always easier to machine the less ductile T6 or T7 heat treated condition, compared to the as cast condition, there is an effect that base metal properties have on machinability that is quite significant. Accordingly, there is not a predictable treatment that improves machinability of hypereutectic aluminum silicon alloys.

Hypereutectic aluminum alloy B391 (AA B391) includes 18 to 20% silicon by weight for wear resistance, 0.4 to 0.7% by weight magnesium for aging response to increase strength and has maximums for iron and copper of 0.2% by weight for good sand casting attributes, and is the only hypereutectic aluminum silicon alloy registered for sand casting by the Aluminum Association. The 0.2% by weight maximum copper constituency ensures that (for any given silicon content), the solidification range, that is, the temperature difference between the liquidus and solidus, is at a minimum. In comparison, AA 390 has the same range of elements as AA B391, except AA 390 has 4.5% by weight copper constituency. Thus, the narrow solidification range of AA B391 occurs primarily because the significantly lower copper constituency raises the solidus melting point by nearly 100° Fahrenheit compared to AA 390.

The narrow solidification range of AA B391 is important because the primary silicon, which is less dense than the molten alloy, it is less likely to float and segregate upon precipitation in an alloy of narrow solidification range. The low iron and manganese contents of AA B391 are desirable and are particularly attractive for a sand cast hypereutectic aluminum silicon alloy that solidifies slowly. The mechanical properties of AA B391 are significantly degraded when the iron phase grows large during the slow cooling, because a needle like morphology results for the iron phase, degrading mechanical properties.

Historically, nickel was an essential element in Y alloy (4% by weight copper, 2% by weight nickel, 1.5% by weight magnesium, balance aluminum), developed during World War I. Nickel is present in only three registered alloys with the Aluminum Association today in concentrations between 2% and 3% nickel. Thus, it is known to use nickel as a minor constituent in some aluminum copper alloys, such as AA 242, AA 336 and AA 393, wherein the element imparts high strength at high temperature. AA 242 has a formulation of 3.7 to 4.5% by weight copper, 1.2 to 1.7% by weight magnesium, 1.8 to 2.3% by weight nickel and balance aluminum. AA 336 has 11 to 13% by weight silicon, 1.2% by weight maximum iron, 0.5 to 1.5% by weight copper, 0.7 to 1.3% by weight magnesium, 2.0 to 3.0% by weight nickel and balance aluminum. Similarly, AA 393 has a hypereutectic formulation of 21 to 23% by weight silicon, 1.3% by weight maximum iron, 0.7 to 1.1% by weight copper, 0.7 to 1.3% by weight magnesium, 2.0 to 2.5% by weight nickel and balance aluminum.

Additionally, more than forty years ago, there was considerable interest in the Al-NiAl₃ eutectic, unidirectionally solidified, as a fiber reinforced material, especially for high temperature applications. As identified in the reference to B. K. Agrawal, Met A 6, 152605, in the book, Aluminum Alloys: Structure and Properties by L. F. Mondolfo page 339 (Butterworth Publications Ltd, 1976), by directional freezing, the eutectic may be made to crystallize with the NiAl₃ fibers aligned in the direction of growth, with the spacing between the fibers dependent on the freezing rate. The same reference indicates that additions of barium, cerium and cesium to the unidirectionally solidified Al-NiAl₃ eutectic changes the solidification pattern from colony to dendritic It is also known that aging after quenching from high temperature does not produce hardening of binary Al-Ni alloys to be of practical use.

However, the addition of nickel in concentrations approaching 6% to aluminum silicon magnesium casting alloys, aluminum silicon copper casting alloys, aluminum silicon copper magnesium alloys or aluminum copper casting alloys have not been studied. This is because it is known that nickel additions of 2% by weight or less have the effect of reducing hot shortness in some castings and also have the effect of reducing the coefficient of thermal expansion.

Additionally, US 6,168,675 B1 describes a hypereutectic aluminum silicon alloy having 2.5 to 4.5% by weight nickel, but with a very high manganese content of 1.2% maximum by weight and a very high iron content of 1.2% by weight maximum. This alloy is intended for the die casting process or permanent mold casting process to make vehicular disk brake components. Because of the high manganese and iron contents, this alloy has a very high heavier metal content that requires a high holding temperature to prevent the heavier metals from dropping out. Furthermore, the high manganese content is necessary to modify the needle like beta iron aluminum phase to the alpha iron aluminum phase and increases the yield strength, tensile strength and elongation, both at ambient and high temperatures. Notwithstanding the attributes imparted to the alloy from high levels of manganese and iron, the alloy of US 6,168,675 B1 would not be suited for a slow cooling process like sand, lost foam or investment casting because the large needle like iron phase particles would form, even with the high levels of manganese, thereby hindering feeding during solidification which results in increased porosity levels and decreased ductility levels.

Sand casting processes are increasingly being used to cast complex metal products. Sand casting procedures include lost foam casting, lost foam with pressure casting, green sand casting, bonded sand casting, precision sand casting and investment casting. Perhaps the most beneficial and economical of these types of castings is lost foam casting with pressure. Such a method is described in US 6,763,876 B1 entitled Method And Apparatus For Lost Foam Casting Of Metal Articles Using External Pressure. All of the above discussion does not mean that die casting alloys containing nickel or nickel-free cannot be made more machinable if the primary silicon particle size is small and the eutectic is modified, which has not heretofore been demonstrated.

Davami P et al. "Strontium as a modifying agent for Al-Si eutectic alloy", British Foundry, Institute of British Foundymen, Chesterfield, GB, Vol. 72, pages 4-7, deals with investigations regarding strontium as a modifying agent.

Dinnis C M et al. "The influence of strontium on porosity formation in Al-Si alloys", Metallurgical and Materials Transactions A, ASM International, Vol. 35A, November 2004, pages 3531-3541, is an investigation regarding the effect of strontium on the amount, morphology, and distribution of porosity in sand castings with marginal solidification conditions.

Barrie S Shabel et al. "Friction and Wear of Aluminum-Silicon Alloys", ASM International 1992, pages 785-794, deals with the wear behavior of aluminum silicon alloys.

The present invention has as an object to provide a hypereutectic high pressure die cast aluminum silicon alloy which has significant structural and microstructural advantages over prior art alloys.

According to the invention the hypereutectic high pressure die cast aluminum silicon alloy comprises 16% to 23% by weight silicon, 0.01% to 1.5% by weight iron, 0.01% to 0.6% by weight manganese, 0.01% to 1.3% by weight magnesium, 0.05% to 0.2% by weight strontium, optionally 0.01% to 4.5% by weight nickel, and the balance aluminum is disclosed. As said, this alloy may include 0.01% to 4.5% by weight nickel, but the nickel constituency may also be omitted. As also said, this alloy may include 0.2% to 5% by weight copper, but the copper constituency may also be omitted.

The iron constituency may be modified to 0.01% to 0.7% by weight iron, or 0.01% to 0.2% by weight iron. The manganese constituency may be modified to 0.01% to 0.5% by weight manganese. The strontium constituency may be modified to 0.05% to 0.1% by weight strontium.

This inventive embodiment, when cooled at high pressure die casting cooling rates, demonstrates significant structural and microstructural advantages. Particularly, the structural advantages include an elongation of at least 2%, an average ultimate tensile strength of greater than 250 MPa, and a yield strength of greater than 200 MPa.

The microstructure of this high pressure die cast aluminum silicon alloy has a volume fraction of primary silicon at greater than 10%, and in one embodiment between 10% to 20%, a volume fraction of modified aluminum-silicon eutectic at 45% to 90%, and the balance of the microstructure primary aluminum. The microstructural advantages include a volume fraction of primary silicon being surrounded by divorced eutectic aluminum, a volume fraction of primary silicon surrounded by a modified eutectic containing a fibrous eutectic silicon phase, and dendritic primary aluminum with an average dendrite arm spacing of less than 15 µm. The volume fraction of primary aluminum, including the modified eutectic that surrounds the aluminum dendrites, is larger than the volume fraction of primary silicon. Also, the primary aluminum dendritic arm spacing is larger than the average silicon particle size.

Preferred modifications and improvements of the alloy according to claim 1 are the subject matter of the dependent claims.

All of the strontium-added embodiments are die casting alloys, and may be die cast while avoiding die soldering using any die casting process, including high pressure die casting (HPDC).

In the following of this description examples for hypereutectic high pressure die cast aluminum silicon alloys are explained in detail with reference to the drawings. In the drawings:
- Fig. 1: demonstrates the binary Al-Si phase diagram.
- Fig. 2: is a ternary diagram for a three phase equilibrium for the Al-Si-NiAl₃ ternary system.
- Fig. 3: is a stress/ strain curve for a well annealed (100 hours at 1000°F) hypereutectic Al-Si nickel free alloy.
- Fig. 4: is the microstructure of an "as cast" phosphorous refined and strontium-free hypereutectic aluminum silicon alloy cast into a permanent mold for tensile specimens.
- Fig. 5: is the microstructure of an "as cast" phosphorous refined, nickel containing but strontium-free hypereutectic aluminum silicon alloy cast into a permanent mold for tensile specimens.
- Fig. 6: is the microstructure of a well annealed (100 hours at 1000°F) "as cast" phosphorous refined and strontium-free hypereutectic aluminum silicon alloy of Fig. 4 cast into a permanent mold for tensile specimens.
- Fig. 7: is the microstructure of a well annealed (100 hours at 1000°F) "as cast" phosphorous refined nickel containing but strontium-free hypereutectic aluminum silicon alloy of Fig. 5 cast into a permanent mold for tensile specimens.
- Fig. 8: is the microstructure of the alloy of present application with 0.05% strontium and demonstrating highly refined primary silicon microstructure; the primary silicon volume fraction is approximately 20%, or nearly twice that of conventional hypereutectic Al-Si alloys, and the primary silicon is surrounded by a divorced eutectic aluminum phase; modified eutectic surrounds primary aluminum dendrites; the volume fraction of primary aluminum is larger than the volume fraction of primary silicon.
- Fig. 9: is the microstructure of a button spectrometer sample (diameter 6.5 cm and 7 mm thick) made by gravity pouring 100 grams of molten AA 391 alloy but with only a 0.016% Sr addition into a permanent mold; the primary silicon particle size is 100 microns.
- Fig. 10: is the microstructure of a button spectrometer sample (diameter 6.5 cm and 7 mm thick) made by gravity pouring 100 grams of molten AA 391 alloy having a 0.030% Sr addition into a permanent mold, and is different than the microstructure of Fig. 8.
- Fig. 11: is a ternary phase diagram for the Al-Si-Fe system, showing the liquidus surface in degrees C.
- Fig. 12: is the microstructure of a button spectrometer sample (diameter 6.5 cm and 7 mm thick) made by gravity pouring 100 grams of a molten alloy having a 0.04% by weight strontium addition.
- Fig. 13: is the microstructure of a button spectrometer sample (diameter 6.5 cm and 7 mm thick) made by gravity pouring 100 grams of a molten alloy having a 0.06% by weight strontium addition.
- Fig. 14: is the microstructure of a button spectrometer sample (diameter 6.5 cm and 7 mm thick) made by gravity pouring 100 grams of a molten alloy having a 0.09% by weight strontium addition.
- Fig. 15: is the microstructure of a button spectrometer sample (diameter 6.5 cm and 7 mm thick) made by gravity pouring 100 grams of a molten alloy having a 0.18% by weight strontium addition.
- Fig. 16: is the microstructure of a button spectrometer sample (diameter 6.5 cm and 7 mm thick) made by gravity pouring 100 grams of a molten alloy having a 0.05% by weight strontium and 4% by weight nickel additions.
- Fig. 17: is an aluminum-silicon phase diagram demonstrating solidification sequences for an alloy exhibiting the microstructure of Fig. 8.
- Fig. 18: is the microstructure of a high pressure die cast bearing carrier spool casting having the following composition by weight percentage: 20.4% Si, 0.65% Mg, 0.26% Fe, 0.07% Cu, 0.04% Mn, 0.022% Sr, and the balance Al.
- Fig. 19: is the binary Al-Ni phase diagram.

Prior to the present invention, the microstructure of hypereutectic aluminum silicon alloys tended to be brittle because phosphorus was required as a nucleus for small primary silicon particle size, and strontium could not be used to modify these eutectic silicon because phosphorus and strontium reacted with one another. Moreover, it was commonly understood that additions of strontium at levels below 0.03% were known to cause the primary silicon particle size to increase, and during machining all of the primary silicon particles would crack and result in very poor castings. The present application surprisingly discovered that if strontium was added in the range of 0.05% - 0.20% by weight to a hypereutectic aluminum silicon alloy, almost all of the primary silicon alloy disintegrated into irregular, small primary silicon particles less than 30 microns in size. The resulting castings exhibited over 2% elongation in the as cast condition because both the primary silicon and the eutectic silicon were respectively, and unexpectedly, refined to a small primary silicon particle size and the eutectic silicon was modified to the fibrous morphology from the acicular morphology by the 0.05% - 0.20% by weight strontium addition. Coupled with these dramatic changes, non -equilibrium primary aluminum dendrites unexpectedly appeared in significant volume fraction in the microstructure with a secondary dendrite spacing [DAS] less than 15 microns. The eutectic structure was so well modified that the eutectic Si and eutectic Al could not be resolved under a microscope at 100X magnification. With the addition of 3 - 6% by weight nickel, further enhances the machinability of the above referenced alloy.

Turning to Figs. 4-7, therein is demonstrated the microstructures from 0.5 inch diameter tensile specimens with a 2 inch gauge length that were made in a standard tensile specimen hinged permanent mold. During gravity pouring of molten metal into the mold, the hinged mold is closed, and extracting of the tensile specimen castings was accomplished by opening the hinged mold after the tensile specimen solidified. The cooling rate in this standard tensile specimen permanent mold is estimated to be 29°C/second, about the same as cooling rate in the 100 gram button spectrometer samples of Figs. 9-10 and 12-16.

Figs. 4-7 are the microstructures of an "as cast" phosphorous refined and strontium-free hypereutectic aluminum silicon alloy cast into a permanent mold for tensile specimens. Figs. 4 and 6 demonstrate the alloy with the following specific constituency: 20% Si; 1.1% Fe; 0.55% Mg; and substantially free of iron copper and manganese (measured at 0% Fe, 0.08% Cu 0.25% Mn). The difference between the micrographs of Figs. 4 and 6 is that Fig. 4 demonstrates the "as cast" alloy, while Fig. 6 demonstrates a well annealed alloy after 100 hours at 1000°F. Figs. 5 and 7 demonstrate the microstructure of the same alloys as Figs. 4 and 6, but with a 4% nickel addition. Similarly, the difference between the micrographs of Figs. 5 and 7 is that Fig. 5 demonstrates the "as cast" alloy, while Fig. 7 demonstrates a well annealed alloy after 100 hours at 1000°F. What is common Figs. 4 through 7 is that the shape morphology of the primary silicon is regular (i.e., the silicon polygons have 4 to six sides), the average primary silicon particle size is about 30 microns because the alloys were phosphorous treated to refine the primary silicon particle size, and the eutectic silicon morphology in the eutectic is acicular or unmodified in the two as cast microstructures. Further, the edges of the primary silicon in the well annealed samples, when compared to the primary silicon in the "as cast" samples, has been rounded by the 100 hours at 1000°F, and this thermal treatment has produced a eutectic silicon that is spherical in shape morphology. The above phosphorous treated microstructures are the baselines that the inventive strontium treated microstructures with be compared to.

The non-nickel alloy of Fig. 4 demonstrated a UTS of 30.0 ksi (or 207 MPa), yield strength of 27.0 ksi (or 186 MPa) and an elongation of 0.5%. The nickel containing alloy of Fig. 5 demonstrated a UTS of 32.2 ksi (or 222 MPa), a yield strength of 28.7 ksi (or 198 MPa) and an elongation of 0.5%. At 400°F (or 205°C) the yield strength of the nickel free alloy drops to 22 ksi (or 155 MPa) from 27 ksi (or 186 MPa), but the nickel containing alloy did not drop but stayed at 28.0 ksi (or 193 MPa). In the well annealed condition (100 hours at 1000°F) to thermally produce the optimal elongation shown in Fig. 6 for the nickel free alloy resulted in a UTS of 17.5 ksi (or 121 MPa), yield strength of 12.0 ksi (or 83 MPa) and elongation of 1.7%. The nickel containing alloy of Fig. 7 when well annealed at 100 hours at 1000°F demonstrated a UTS of 18.0 ksi (or 124 MPa), yield strength of 12..3 ksi (or 85 MPa) and an elongation of 1.7%. Accordingly, the well annealed samples produce an elongation baseline for the inventive strontium containing die casting alloys.

For the high pressure die casting process, a desirable primary silicon size is 20 microns. This desirable microstructure requires the primary silicon to be phosphorous refined. That is, it requires the creation of copious nucleation sites of aluminum phosphide and the fast cooling rate of die casting (i.e., 80°C/sec). A problem arises because strontium phosphide or sodium phosphide compounds are more stable thermodynamically than aluminum phosphide and thus a rapid coarsening of the primary silicon occurs if strontium or sodium is present in the melt in greater concentration than the phosphorous. Moreover, a 50 micron primary silicon particle sized particle generally cracks extensively during machining. Thus, a 25-35 micron particle size in high pressure die casting is the goal.

In Fig. 4, the primary silicon particle size is 20 to 60 microns, with an average of about 30 microns. The eutectic silicon morphology is acicular (or not modified, and thus not fibrous or modified). The 300 ppm phosphorous caused single nucleation of the silicon on each of the many created aluminum phosphide (AIP) particles which resulted in the regular shaped morphology of the primary silicon particles. The coating on the permanent mold die slowed the cooling of the casting compared to the high pressure die casting process resulting in an average primary silicon particle size of about 30 microns and an elongation of 0.5%.

By adding 4% by weight nickel to the alloy of Fig. 4, the microstructure of Fig. 5 is achieved. The primary silicon particles have a blocky regular morphology and the primary silicon particle size is 20 to 60 microns, with an average of about 30 microns. The eutectic silicon morphology is acicular (not modified or fibrous) and the ternary eutectic NiAl₃ phase (located mainly in lower right hand corner) is not the primary NiAl₃ phase. The phosphorous caused the single nucleation of the silicon on the created AIP particles and the regular shaped particles. Again, the coating on the permanent mold die slows down the cooling of the casting compared to the high pressure die casting process and results in an average primary silicon particle size of about 30 microns and an elongation of 0.5%.

Turning now to Figs. 6 and 7, the nickel containing alloy in Fig. 7 has significantly smaller eutectic silicon particles than the eutectic silicon particles in the nickel free alloy in Fig. 6. However, even more important is that in Fig. 7 for the nickel containing alloy, the eutectic NiAl₃ particles are smaller than the eutectic silicon particles, and much smaller than the eutectic silicon particles in Fig. 6 for the nickel free alloy. This is quite significant microstructural because it is apparent that at 100 hours at 1000°F the temperature was high enough to break down both the eutectic silicon phase and the eutectic NiAl₃ phase and cause growth of the eutectic silicon phase but not the growth of the eutectic NiAl₃ phase. As a result, the nickel containing alloys have higher temperature properties.

Throughout this application mechanical properties are reported. Fig. 3 shows a typical chart generated when tensile tests are performed. More specifically, Fig. 3 is the stress strain curve for well annealed (100 hours at 1000°F) nickel free alloy. The stress in units of ksi is identified on the vertical axis and the strain % is on the horizontal axis. The slope of the red line is the Modulus of Elasticity, and where the slope of the 0.20% off-set blue line intersects the stress strain curve is the yield strength. The stress where the tensile specimen fails is the Ultimate Tensile Strength (or UTS).

There is a further significance in these results in that 100 hours at 1000°F was more than sufficient to break down the eutectic NiAl₃ phase which improves mechanical properties but not sufficient in breaking down the much larger primary NiAl₃ phase. Accordingly, the nickel containing alloy of the present application with strontium, and having the ternary eutectic NiAl₃ phase in the microstructure but no primary NiAl₃ phase in the microstructure, has significant potential for use in many different types of castings.

Further unexpected results occurred when strontium in the range of 0.03 to 0.2% by weight was added to the alloys. Fig. 8 demonstrates the "as cast" microstructure of tensile specimens extracted from a cast engine block having the following specific constituencies: 19.2% by weight Si; 0.05% by weight Sr; 0.7% by weight Fe; and 0.46% by weight Mg, with the balance aluminum. The alloy was substantially free of copper and manganese (measured at 0.09% Cu and 0.24% Mn) and only an incidental amount of nickel was found at 0.05% by weight Ni. Testing of three specimens from this casting revealed an average UTS of 38.1 ksi (263 MPa), a yield strength of 30.0 ksi (207 MPa) and an elongation of 2.1%, which is four times the elongation of a typical hypereutectic Al-Si alloy of 0.5%, and longer than the elongation of a well annealed conventional hypereutectic Al-Si alloy.

In Fig. 8, the form of the primary silicon is unexpectedly not "regular" but smaller and irregular, presenting the opportunity for better machining because the primary silicon is refined and small in size, with an average size less than 10 microns or smaller than the better than best results expected in conventional phosphorous refined primary silicon in high pressure die casting. Further, there is a large fraction of primary silicon for high wear resistance. Moreover, the eutectic is unexpectedly modified most likely through a very large undercooling that produces a secondary dendrite arm spacing (SDAS) of 10 microns or less for the primary aluminum dendrites along with a significant higher volume fraction of primary aluminum dendrites and fibrous modified eutectic silicon that cannot be resolved in the eutectic between the clusters of disintegrated primary silicon particles.

Typically, the primary silicon phase of hypereutectic Al-Si alloys is not readily nucleated by impurities present in these alloys. As a result, phosphorous is added to hypereutectic Al-Si alloy melts in permanent mold casting, and very frequently in die casting for nucleation. As noted above, the phosphorous (in amounts of about 100 to 500 ppm) reacts with the liquid aluminum to form AIP, which has a crystal structure very similar to that of silicon, and acts as an effective heterogeneous nucleant. Strontium phosphide and sodium phosphide, however, are compounds that are more stable than aluminum phosphide and therefore a coarsening of the primary silicon is expected when strontium or sodium is added to the melt.

The microstructure in Fig. 9 illustrates the accepted scientific logic of this reasoning (i.e., adding strontium increases the primary silicon size). By adding 0.016% strontium, the primary silicon size tripled in size. Fig. 9 demonstrates that under 0.03% by weight strontium, the hypereutectic alloy has the regular blocky primary silicon particles size morphology of 90 microns in size. As shown in Fig. 9, strontium levels typical of those required to cause modification in hypoeutectic alloys like A356 coarsen the primary silicon, but the primary silicon retains its blocky regular shape morphology. Compared to the phosphorous refined primary silicon size of 30 microns produced in Figs. 4-7 with 0% strontium that exhibited no chemical modifications of the eutectic silicon, at 0.016% strontium, modification of the eutectic silicon phase is effected, and the primary silicon morphology retains its blocky regular shape morphology, but a big price is paid, the primary silicon size here is three times larger at 90 microns and the elongation is still 0.5% or less. Indeed, adding strontium from 0.001 % to just below 0.03% increases the size of the primary silicon particles, as shown in Fig. 9. Thus, one of ordinary skill in the art would expect the primary silicon size to continue to increase as the strontium addition is increased. However, what was surprisingly found, and what is demonstrated in Figs. 8, 10 and 12-16 is that when strontium is added at 0.03% by weight and above, the primary silicon fragments and disintegrates, as if it exploded, to a smaller primary silicon particle size with an irregular shape morphology and the eutectic silicon is modified.

As seen in Fig. 8, with the strontium addition of 0.05 to 0.2% by weight, the micrograph exhibits a microstructure with a refined primary silicon particle size less than 15 microns. This is almost half the best silicon particle size produced in conventional die casting with phosphorous refinement of the primary silicon. Unlike the microstructure in Fig. 9 with strontium at 0.016%, the microstructure in Fig. 8, demonstrates individual starting primary silicon particle appears to be fragmented into four or five smaller pieces of less than 15 microns. Moreover, the alloys of the present invention demonstrate a modified eutectic with the eutectic silicon morphology that is fibrous in nature. The combination of both a refined primary silicon and a modified eutectic silicon has not been exhibited in production castings heretofore and is responsible for elongations in production parts that exceed 2% elongation, i.e., four times the elongation of strontium-free conventional hypereutectic Al-Si alloys.

Further, in a typical hypereutectic 391 alloy with 18-20% silicon, the equilibrium weight fraction of alloy that freezes as eutectic is approximately 91%. This is much greater than the approximately 9% that solidifies as primary silicon. With the present invention, modification of the eutectic silicon in the eutectic with strontium affects considerably more of the micro-constituent representing 91% of the alloy weight than does primary silicon refinement with phosphorus which represents 9% of the alloy weight. This 10 to 1 ratio driving the modification of the eutectic silicon in the eutectic, at least as far as the tensile properties are concerned, can more than compensate for the expected considerable coarsening of the primary silicon phase. Significant increase in UTS (25%), yield strength (10%), elongation (400%) and quality index (250%) were found by the inventors when the eutectic silicon is modified in accordance with the present invention. One of skill in the art will recognize, however, that machinability becomes more of a problem with a coarse primary silicon, if the die casting process is not used, and if the 4% nickel alloy, having the ternary eutectic NiAl₃ phase, is not used.

Figs. 10 and 12-16 also demonstrate visible eutectic cells because the cell boundaries appear to be decorated with sub-micron sized Al₄Sr particles. The smallest eutectic cell size is about 65 microns and the largest about 200 microns, while the average is about 100 microns. In the ever changing eutectic modification theory, the currently accepted theory is that eutectic silicon modification is accompanied by a tenfold increase in the cell size for hypoeutectic Al-Si alloys, according to S.D. McDonald in his Ph.D. thesis from University of Queensland, Brisbane, Australia, July, 2002. However, this cell size can only be seen in hypoeutectic Al-Si-Cu[-Fe] alloys wherein the cell boundaries are decorated with either the CuAl₂ phase or beta platelets of the Al₅FeSi phase. Thus, the accepted theory of modification of hypoeutectic Al-Si alloys never mentioned the eutectic cell size in any technical explanation until 2002 because evidence of the cell size was never observed until 2002, and only after the development of very special techniques to see eutectic cell grains in Al-Si alloys. As the ternary phase diagram for the Al-Si-Fe system shown in Fig. 11 indicates, beta (β) phase platelets of the Al₅FeSi phase in hypoeutectic Al-Si-Fe alloys can be explained if the iron is 1% or higher and the silicon is 13%, but it is impossible for them to form in the higher silicon hypereutectic alloys. The ternary phase diagram suggests that the delta (δ) iron phase might precipitate in Al-Si with more than 14% or higher Si but this has never been reported. The phase diagram of Fig. 11 indicates that at 1% Fe and 14% Si, the β iron Al₅FeSi and the δ iron phase cannot form if the iron is less than 1%. This suggests that the phase that decorates the eutectic cells is Al₄Sr, by a process of elimination.

Visible eutectic cells in the permanent mold cast specimens are mentioned because no special technique was used to see the eutectic cells in Figs. 10 and 12-16. The microstructures are simply polished samples with no enchant required. It is believed that the small species that very clearly decorate eutectic cell boundaries in Figs. 10 and 12-16 are most probably the Al₄Sr phase particles. Further, the eutectic cells are clearly seen in these figures are samples with more than 0.03% strontium cooled at 29°C/sec, and are associated with the small broken up irregularly shaped silicon particles and a modified eutectic structure. However, two important observations are apparent when compared to Fig. 8. First, there is an absence of undercooling, non-equilibrium primary aluminum phase in Fig. 10. Second, there is the absence of the very small primary silicon phase (in Figs. 10 and 12-16), which clearly are visible in the Fig. 8 microstructure of the high pressure die cast block that cooled at 60 or more °C per second, more than twice the cooling rate of the button spectrometer samples. On closer examination of the high pressure die cast microstructure in Fig. 8 compared to the permanent mold microstructure in Figs. 9 or 10 and 12-16, is the absence of what is believed to be the Al₄Sr phase in Fig. 8 and presents in the other cited figures, suggesting the high pressure die casting cooling rate is needed to suppress the precipitation of the speculated Al₄Sr phase. At the lower cooling rates of sand casting, the microstructure of the button spectrometer sample containing 0.03% Sr or more have the large dendritic morphology of the primary silicon particles seen in Figs. 10 and 12-16, whereas Fig. 8 has small irregular shaped primary silicon particles, further suggesting the cited microstructures are cooling rate dependent, and the die casting cooling rate produces the preferred microstructure.

For specificity, the particular constituencies of the hypereutectic aluminum silicon alloys shown in Figs. 8-10 and 12-16 are provided in Table 1, below. Note that the constituencies represent positive additions to the alloys, rather than impurities from the stock metals. Further, all alloys contain Aluminum as the balance constituency.

| **Figure** | **% Silicon** | **% Strontium** | **% Nickel** | **% Magnesium** | **% Iron** | **Impurities** |
|---|---|---|---|---|---|---|
| 8 | 19.2 | 0.050 | 0 | 0.46 | 0.7 | 0.09 Cu, 0.24 Mn, 0.05 Ni |
| 9 | 18.5 | 0.016 | 0 | 0.59 | 0.6 | 0.17 Cu, 0.19 Mn, 0.02 Ni |
| 10 | 18.4 | 0.030 | 0 | 0.59 | 0.6 | 0.17 Cu, 0.18 Mn, 0.01 Ni |
| 12 | 18.4 | 0.040 | 0 | 0.58 | 0.6 | 0.16 Cu, 0.19 Mn, 0.01 Ni |
| 13 | 18.5 | 0.060 | 0 | 0.57 | 0.6 | 0.17 Cu, 0.18 Mn, 0.01 Ni |
| 14 | 18.4 | 0.090 | 0 | 0.57 | 0.6 | 0.16 Cu, 0.18 Mn, 0.01 Ni |
| 15 | 18.5 | 0.18 | 0 | 0.57 | 0.6 | 0.16 Cu, 0.19 Mn, 0.01 Ni |
| 16 | 18.5 | 0.05 | 4.3 | 0.56 | 0.6 | 0.16 Cu, 0.18 Mn, |
| 18 | 20.4 | 0.022 | 0 | 0.65 | 0.26 | 0.07 Cu 0.04 Mn |

The results of the alloy made in accordance with the present invention is a complex microstructure with a majority of the primary silicon particles with a particle size of less than 15 microns. Moreover, the eutectic structure is modified, with the primary aluminum phase in the microstructure with a secondary dendrite arm spacing of less than 15 microns. Further, the primary silicon volume fraction is about 20% (twice that found in normal hypereutectic Al-Si alloys) and these primary silicon particles are surrounded by a divorced eutectic aluminum. The modified eutectic surrounds the primary aluminum dendrites. The volume fraction of primary aluminum dendrites, including the modified eutectic that surrounds the primary aluminum, is larger than the volume fraction of the primary silicon including the divorced eutectic aluminum that surrounds the primary silicon, and the secondary dendrite arm spacing of the aluminum is larger than the primary silicon particle size. The alloys also have an elongation of 2.1% for the "as cast" sample of Fig. 8, and this is four times the typical elongation of 0.5% in "as cast" conventional hypereutectic Al-Si alloys. This elongation is also higher than the elongation that can be obtained in well annealed conventional hypereutectic Al-Si alloys. At higher temperatures, e.g., 400°F, the nickel containing alloy has higher mechanical properties.

The alloy may have a T6 heat treated microstructure of primary silicon particles embedded in a eutectic of Al-Si or Al-Si-NiAl₃ and is generally free of unsolutionized Mg₂Si phases and Cu₃NiAl₆ in Chinese script compacted blocky morphology form. The hypereutectic aluminum silicon alloy has an anticipated use with a die casting process to cast engine components such as engine blocks, engine heads and pistons, particularly when such components are to be used in salt water where high corrosion resistance is required. The alloy provides high mechanical properties (through low porosity levels) both at ambient temperatures and at elevated temperatures.

Achieving high corrosion resistance and low porosity levels necessitates an alloy composition low in copper content. Copper is extensively soluble in aluminum, reaching 5.65% at the binary Al-Si eutectic temperature and, as a result, copper destroys the corrosion resistance of aluminum to a greater extent than any other common element in the periodic table. Aluminum silicon alloys containing copper precipitate the copper containing phases at low temperatures late in the solidification process after the precipitation of the primary aluminum phase. This low temperature, late precipitation event clogs the interdendritic feed passageways created by the primary aluminum silicon dendritic. As a result, the copper containing aluminum silicon alloys cast with the lost foam casting process of US 6,763,876 B1 typically contain ten times the level of porosity that can be obtained with the copper free aluminum silicon alloys.

The present invention describes system engineered design changes based on the introduction of the NiAl₃ phase into an aluminum silicon eutectic microstructure. These design changes provide partitions in the aluminum silicon eutectic that increase machinability and provide an intermetallic compound constituent in the eutectic having greater galvanic couple compatibility in a salt water environment than with aluminum-nickel or aluminum-silicon.

Clogging of the interdendritic passageways for alloys with high iron constituencies (e.g., AA 336 and AA 393) may occur because the iron phase forms long, needle like phases during solidification, clogging the interdendritic passageways and causing the alloy to have high microporosity. In contrast, the "Chinese script" compacted, blocky phase morphology of an NiAl₃ eutectic phase is blocky but compacted and intermixed with aluminum silicon eutectic when formed under die casting cooling rates in the ternary reaction (Liq > Si + Al + NiAl₃). Significantly, the coarse NiAl₃ primary phase starts to precipitate, particularly for Ni compositions above 6%, before the ternary eutectic temperature is reached. Thus, nickel contents above 6% should be avoided if mechanical properties, and in particular ductility, is important. The NiAl₃ network in the ternary eutectic, because of its open structure at the micron level, is quite permeable for the liquid constituents that do not contain solid copper phases or solid iron phases and thus, this morphology does not hinder the interdendritic feeding of molten aluminum. As a result, hypereutectic aluminum -silicon alloys containing nickel, but having low levels of both iron and copper, have lower porosity levels, when high pressure die cast with pressure intensification.

During solution heat treating of "as cast" samples, there is a clear difference between copper containing hypereutectic aluminum silicon alloys with nickel and copper free hypereutectic aluminum silicon alloys with nickel. Solution heat treating solubilizes Mg₂Si and most of the Cu₃NiAl₆ phase, but only causes simple rounding of the silicon and NiAl₃ particles, as seen in Figs. 6 and 7. The phenomenon occurs because silicon and NiAl₃ are basically insoluble in aluminum, while magnesium and copper are extensively soluble in aluminum. Thus, results suggest that silicon and NiAl₃ should provide strength and stability at elevated temperatures to a greater extent than magnesium, copper and manganese. The results also suggest that microstructures obtained with the copper free aluminum silicon alloys containing nickel are relatively stable at room temperatures after slow cooling through the solidification event, because no non-equilibrium phases form. Fast cooled samples, on the other hand, because of the possible presents of non-equilibrium phases (such as, primary aluminum dendrites in a hypereutectic aluminum-silicon alloy, as in Fig. 8), might be expected to have microstructures that have unique advantages at room temperatures, and if nickel is a constituent in the non-equilibrium phase, that phase may have stability at an elevated temperature also.

Additionally, it has been realized that when nickel is added to the eutectic constituents as an NiAl₃ compound rather than as a pure element (that is insoluble in aluminum), there is no uncombined nickel (i.e., "free nickel") present in the microstructure. This is significant because free nickel affects galvanic corrosion phenomena adversely, while NiAl₃, as aforementioned, has beneficial effect of facilitating corrosion resistance.

It is known that in man-made metal matrix composites, the volume fraction of the reinforcing phase is increased by artificially adding more of the reinforcing phase. With eutectics, the volume fraction of the reinforcing phase (i.e., the "fiber phase") and the matrix phase are fixed by nature by the eutectic composition and by the compositions of the phases in equilibrium at the eutectic temperature.

The AA B391 alloy is associated with a binary Al-Si eutectic that has a long arrest temperature isotherm at 577° Celsius. The long arrest isotherm allows liquid styrene to escape when cast in the lost foam casting process, which has the effect that it is less likely that liquid styrene defects will be in lost foam castings. Particularly with nickel, under equilibrium conditions there should be only one arrest temperature, and that is the ternary eutectic temperature of the Al-Si- NiAl₃ at 557°C for the 5% Ni alloy, 20°C below the Al-Si eutectic temperature. However, under the non-equilibrium cooling conditions of high pressure die casting, the arrest temperatures of the Al-Si eutectic at 577°C and of the Al-Ni eutectic at 640°C may also come into play. Thus, the microstructure in Fig. 8. The non-equilibrium arrest temperatures are expected to enhance feeding of shrinkage porosity. Copper containing aluminum silicon alloys with nickel, in addition to the above, would also contain the Cu₃NiAl6 phase in Chinese script compacted blocky form that would aid in machinability but would contain low melting copper phases that precipitate late in the solidification process and clog the feed passageways, preventing the attainment of low porosity levels.

The copper free hypereutectic aluminum silicon alloys, with a solidus melting point of nearly 100° Fahrenheit higher than the copper containing hypereutectic aluminum silicon alloys, do not precipitate low melting point phases that clog the interdendritic passageways feeding this shrinkage porosity. Thus, the coarse Chinese script morphology of the NiAl₃ phase in the Al-NiAl₃ eutectic, when solidified under sand casting cooling rates, enhances the feeding of shrinkage porosity because of the NiAl₃ size and morphology relative to the eutectic silicon phase.

Accordingly, the NiAl₃ is preferably introduced into the eutectic and does not materially change the initial primary silicon volume fraction. Further, the NiAl₃ addition imparts high wear properties because long tie lines from essentially pure silicon to the Al-Si eutectic equilibrium remain relatively constant. However, the NiAl₃ addition increases the volume fraction of the eutectic constituents, and accordingly, less Al-Si eutectic must freeze at the lowest temperatures. This is advantageous because, compared to a normal binary eutectic, all of the solidification does not have to occur at one temperature.

Accordingly, there is a lengthened time frame with an organized sequence of solidification events over a range of temperatures. The job of "feeding" shrinkage (e.g., with the pressure intensification of high pressure die casting) is improved. This is beneficial to the quality of the casting as defects are reduced. Accordingly, because the alloy with the NiAl₃ compound addition creating either a binary Al-NiAl₃ eutectic equilibrium or a ternary Al-Si-NiAl₃ eutectic that occur at a higher temperature than the Al-Si eutectic, effectively the temperature of the eutectic is raised and the viscosity of the melt is increased by 10 to 15%.

Thermodynamically, the heat fusion of aluminum is quite high at 92.7 calories per gram, while the heat of fusion of NiAl₃ is 68.4 calories per gram. However, the heat of fusion of silicon is much higher at 430 calories per gram, nearly five times that of aluminum and over six times that of NiAl₃. Thus, as a nickel free hypoeutectic aluminum silicon alloy solidifies and gives off 430 calories per gram as the primary silicon precipitates, there is a tendency for the temperature gradient on the aluminum to decrease. The decrease of the temperature gradient of the aluminum reduces the heat input to the melt and causes shrinkage porosity to become more difficult to feed. Thus, nickel containing Al-Si alloys should feed porosity better than nickel-free Al-Si alloys.

In contrast, as the hypereutectic aluminum silicon alloy solidifies and NiAl₃ precipitates out of solution, only 68.4 calories per gram of heat are given off. Thus, during this early stage of solidification when NiAl₃ is precipitating out of the solution, a larger temperature gradient is expected and, as a result, the feeding efficiency of the shrinkage porosity is greater than when compared to an alloy without nickel. The addition of the NiAl₃ compound thus provides favorable conditions for decreasing the amount of eutectic liquid that will have to go through the Al-Si eutectic during the last stages of solidification for the alloy, and further increasing shrinkage porosity feeding efficiency.

Magnesium is present in the alloy of the present invention for its age hardening response. Under the conditions of equilibrium for hypereutectic aluminum silicon alloys, Mg₂Si does not appear visible at less than 2000X magnification in the as cast condition as a coarse constituent of the eutectic until a magnesium content of about 0.75% has been attained. Also, when the magnesium level is kept below 0.75%, aluminum, silicon and Mg₂Si form a ternary eutectic containing 4.97% magnesium, and 12.95% silicon and freezes at 555° Celsius.

Silicon is present in the proposed alloy for the wear resistance properties imparted by the hard primary silicon particles.

Silicon levels higher than 20% by weight will contain 100% more primary silicon particles than a 16% by weight silicon alloy, but are not advised because the liquidus is above 700° Celsius.

The electrolytic potential of the NiAl₃ compound is negative 0.73 volts, as compared with negative 0.85 volts for pure aluminum. The potential of aluminum-nickel alloys decreases slowly from pure aluminum to NiAl₃. Metals with large positive standard electrode potentials (e.g., Au, Ag, Cu) show very little tendency to dissolve in water and are known as noble metals. However, base metals with a negative standard electrode potential have a tendency to dissolve in water or corrode, such as magnesium and sodium. Thus, a galvanic couple between aluminum and NiAl₃ shows a slight tendency of the less noble aluminum metal in the system to dissolve in the electrolyte. The galvanic corrosion of aluminum coupled to pure nickel would be expected to be far worse because nickel is significantly more noble than NiAl₃. Thus, since the nickel is entirely tied up in the NiAl₃ compound, the addition of nickel to the alloy does not decrease the alloy's application for salt water use. In fact, the potential difference for the Al-NiAl₃ couple in salt water is less than the potential difference for the Al-Si couple in salt water.

Pistons are the engine components that require the highest elevated temperature properties. A low thermal expansion coefficient is of paramount importance in selecting a material for piston construction. Nickel decreases the thermal expansion coefficient of aluminum to a greater extent than any other element and, at a 6% nickel addition, the thermal expansion coefficient of aluminum decreases by approximately 10%. High thermal conductivity is also a very important property for piston construction because the combustion heat of the engine must be dissipated. However, elements that dissolve in aluminum in the solid state solution affect the lattice structure and decrease the thermal conductivity of aluminum. Accordingly, heat treating procedures that cause the precipitation of phases from solution in aluminum, such as the T5 heat treatment versus the T6 heat treatment, is the appropriate heat treatment for an aluminum piston alloy.

It is known that nickel is insoluble in aluminum in the solid state. Nickel has no measurable effect on the thermal conductivity of aluminum because the maximum solubility of nickel and aluminum is approximately 0.04%. Nickel forms a eutectic with aluminum at the aluminum end of the Al-Ni binary diagram. The Al-Ni eutectic requires a liquid alloy of approximately 6% by weight nickel to decompose at 640° Celsius on cooling to a mechanical mixture of basically "pure" solid aluminum and NiAl₃. This solidified alloy has a density of approximately 2879 kg/m3. This density is less than the expected algebraic calculated density of 3072 kg/m3 for a 6% addition of nickel because the NiAl₃ expands upon solidification.

Referring now to the Al-Si phase diagram of Fig. 1 and the Al-Ni binary phase diagram of Fig. 19, although a phase equilibrium diagram for the Al-Si-NiAl₃ ternary system does not exist, it will be recognized by those skilled in the art that a ternary eutectic transformation liquid > Al + NiAl₃ + Si occurs at approximately 5% Ni, 11-12% Si at 557°C. In the solid state the three phases Al, NiAl₃, and Si are present in most of the alloys. The solubility of silicon in NiAl₃ is of the order of 0.4-0.5%; the solubility of nickel in aluminum is only 0.04% at the binary eutectic temperature and that of silicon is reduced by nickel additions. This knowledge, combined with the Al-Sl phase diagram of Fig. 1 and the Al-Ni phase diagram of Fig. 19 demonstrates that there is a three phase equilibrium for the Al-Si-NiAl₃ ternary system. Thus, a ternary diagram may be constructed demonstrating that equilibrium occurs over a temperature range and not, as in binary systems, at a single temperature, as demonstrated in Fig. 2. According to the Gibbs' Phase Rule, the three phase equilibrium in the ternary system is bivariant. The Gibbs' Phase Rule states that the maximum number of phases (P) that can coexist in a chemical system or alloy, plus the number of degrees of freedom (F) is equal to the sum of the components (C) of the system plus 2. Thus, in the Al-Si-NiAl₃ equilibrium, two degrees of freedom exists because there is a maximum number of 3 phases that can coexist and 3 components of the system exist since F=(C+2)-P according to the Gibbs' Phase Rule. Accordingly, after the pressure has been selected, only the temperature or one concentration parameter need be selected in order to fix the conditions of equilibrium.

The representation of a three-phase equilibrium on a phase diagram requires the use of a structural unit that will designate, at a given temperature, the fixed composition of three conjugate phases (i.e., the Al phase, the Si phase and the NiAl₃ phase). The structural unit is found in the "tie triangle" of Fig. 2, where R represents the Al phase, S represents the NiAl₃ phase and L represents the Si phase. The triangle R-S-L connects the three phases that the original phase P decomposes into. Using P as the experimental condition 20% Si, 6% Ni and approximately 73% Al, and using the formulas, tabulated in Fig. 2, to calculate the percentage of NiAl₃ and percentage of silicon, the percentage of NiAl₃ is determined to be 11% and the percentage of silicon is determined to be 8%. These calculations are in reasonable agreement (i.e., + or - 1% for NiAl₃ and + or - 0.5% for silicon) with quantitative metallography that was measured on ten samples.

It has been observed that the NiAl₃ phase precipitates out of the high pressure die casting alloy at about a 14% quantity as a semi-continuous mass of "Chinese script" compacted blocky phases in the eutectic structure between primary silicon particles and primary aluminum dendrites. Meanwhile, the primary silicon volume fraction is approximately 8% in typical sand cast microstructure. This unique microstructure is particularly important for improved machinability and further provides the appropriate reinforcement for elevated temperature creep strength and other elevated temperature properties, making the alloys of the present invention an excellent choice of material for piston construction.

According to the present invention, a hypereutectic aluminum silicon high pressure die cast alloys is disclosed herein having 16% to 23% by weight silicon, 0.01% to 1.5% by weight iron, 0.01% to 0.6% by weight manganese, 0.01% to 1.3% by weight magnesium, 0.05% to 0.20% by weight strontium and the balance aluminum. This alloy may also include 0.01% to 4.5% by weight nickel and 0.2-5% Cu as optional additions.

The iron constituency may be modified to 0.01% to 0.7% by weight iron, or 0.01% to 0.2% by weight iron. The manganese constituency may be modified to 0.01% to 0.5% by weight manganese. The strontium constituency may be modified to 0.05% to 0.1% by weight strontium. This embodiment, when cooled at high pressure die casting cooling rates, demonstrates significant structural and microstructural advantages.

Alloys of this embodiment are substantially free of copper, and thus have a higher solidus temperature and a narrower solidification range than copper-containing hypereutectic Al-Si alloys like AA390 and AA392. This contributes to a more uniform distribution of the primary silicon and improved wear resistance. The higher solidus temperature of the alloys of this embodiment is approximately 85°F higher than the copper-containing alloys. Alloys of this embodiment exhibit over 2% elongation. In comparison, AA390 and AA392 exhibit elongations of 0.5%, due to a relatively large primary silicon particle size and an unmodified eutectic. AA390 and AA392 are used in the manufacture of linerless all-aluminum engine blocks. However, these alloys are also used in the manufacture of pistons and other structural parts, which require a certain level of damage tolerance not adequately supplied by a brittle alloy. Thus, there is a need for hypereutectic Al-Si alloys with a higher solidus melting temperature and greater ductility. Alloys of the presently discussed embodiment having a microstructure consisting of primary aluminum dendrites, surrounded by both a strontium modified-eutectic structure and a refined primary silicon phase, can meet this need.

Normally, a hypereutectic Al-Si-Mg alloy consists of 90% or more eutectic and 10% or less primary silicon, the alloys of this embodiment causes the volume fraction of the eutectic to be partitioned, in a manner never before exhibited, into a higher silicon constitute, more primary silicon (surrounded by aluminum), and a lower silicon constitute, primary aluminum surrounded by a modified eutectic. The increase in volume fraction of primary silicon of small size increases the wear resistance, and the significant decrease in the eutectic volume fraction to primary aluminum (surrounded by modified eutectic) increases the ductility.

Referring now to Figure 8, therein is shown a micrograph of the microstructure from a high pressure high pressure die cast engine block made from an alloy of this embodiment. As noted, the specific constituencies for this alloy are 19.2% by weight Si; 0.05% by weight Sr; 0.7% by weight Fe; and 0.46% by weight Mg, with the balance aluminum. It was unexpectedly found that hypereutectic aluminum silicon alloys with 0.05% to 0.10% strontium, when high pressure die cast, exhibit a microstructure with a refined primary silicon particle size less than 10 microns (µm). Typically, in the high pressure die casting process, a desirable primary silicon size is 20 µm. Accordingly, the small silicon particle size exhibited in the alloy of the present embodiment is nearly half the best size produced in die casting with phosphorous refinement of the primary silicon.

The alloys of this embodiment also demonstrate a modified eutectic with a eutectic silicon morphology that is fibrous in nature. Additionally, be a very large undercooling that produces dendritic primary aluminum with a dendrite arm spacing of 10 microns or less. This undercooling also produced an alpha aluminum halo around and between the primary silicon, because of a divorced eutectic reaction. As a result, an alloy of this embodiment will have a volume fraction of primary aluminum dendrites surrounded by a modified eutectic that is larger than the volume fraction of primary silicon surrounded by a divorced eutectic aluminum. The primary aluminum dendrites with a dendritic arm spacing of 10 microns or less, and the fibrous modified eutectic silicon in between the dendrite arm spacing and entirely around the aluminum dendrites are unexpected. These unique features have not been exhibited in production castings heretofore and are responsible for elongations in production parts that exceed 2% elongation, i.e., four times the elongation of strontium-free conventional hypereutectic Al-Si alloys. Specifically, standard testing revealed that the alloy had average ultimate tensile strength (UTS) of 263 MPa (or 38.1 ksi), a Yield Strength of 207 MPa (or 30.0 ksi) and an elongation of 2.1%. The elongation is four times the elongation of a typical hypereutectic Al-Si alloy of 0.5%, and higher than the elongation of a well annealed conventional hypereutectic Al-Si alloy.

Referring back to Fig. 8, the microstructure shown there consists of (1) small closely spaced irregular shaped silicon particle embedded in an aluminum matrix (because of a divorced eutectic reaction) and (2) larger aluminum dendrites embedded in a modified eutectic. The majority of the "primary" silicon particles are rather concentrated with very little space between the particles. This space between or around the silicon particles is effectively an aluminum alloy halo of very low silicon content. The area of the concentrated patches of many silicon particles with aluminum halos is less in area than the area of the primary aluminum dendrites that are embedded in the modified eutectic. With the majority of the primary silicon particles with a serrated appearance very close to one another and having a small particle size of less than 10 µm, it is clear that these particles never come in contact with each other because of the aluminum halo around the silicon particles. Thus, the silicon never fractures but effectively rejects the aluminum from the high silicon areas during solidification.

These smaller primary silicon sized particles, surrounded by pure aluminum, as a result of the divorced eutectic reaction, accounts for the elongation being four times the elongation of convention hypereutectic Al-Si alloys. The good ductility associated primary aluminum is effective because between the dendritic arm spacing and around the entire primary aluminum dendrite the eutectic structure is modified.

Typically, the primary silicon phase of hypereutectic Al-Si alloys is not readily nucleated by impurities present in these alloys. As a result, phosphorous is consistently added to hypereutectic Al-Si alloy melts in permanent mold casting, and very frequently in die casting. The phosphorous, in amounts of about 100 to 500 ppm, reacts with the liquid aluminum to form aluminum phosphide, AIP, which has a crystal structure very similar to that of silicon, and acts as an effective heterogeneous nucleation site for the primary silicon. Strontium phosphide and sodium phosphide, however, are compounds that are more stable than aluminum phosphide and therefore a coarsening of the primary silicon is expected when strontium or sodium is added to the melt. The microstructure in Figure 9 illustrates the scientific accepted logic of adding 0.016% strontium and having the primary silicon size, as expected, tripled in size. Adding more strontium in Fig. 10 to the 0.03% Sr level, which does not make sense to do based on Fig. 9, should further increase the primary silicon size, but instead resulted in irregularly shaped smaller primary silicon. Thus, an elongation of 2% and larger was found for a strontium content at 0.05% only for die casting cooling rates and not for permanent mold casting cooling rates. The optimal microstructure of Fig. 8 logically has to arise because the freezing process is not an equilibrium process but a quasi-equilibrium process, as suggested schematically in Fig. 17.

Referring now to Fig. 17, the primary silicon phase in conventional hypereutectic aluminum silicon alloys nucleates with the help of an aluminum phosphide particle at A below the liquidus temperature, and then begins to grow as the temperature follows the arrows to B where the unmodified eutectic forms. Similarly, in conventional hypoeutectic aluminum silicon alloys containing strontium the primary aluminum phase forms along the C-curve and grows as the temperature decreases until B is reached and a unmodified eutectic forms. Since the presence of strontium poisons the aluminum phosphide nucleus in hypereutectic aluminum silicon alloys, the primary silicon particles grow to large sizes and crack on machining. With the fast cooling rates of high pressure die casting applied to a hypereutectic aluminum silicon melt with no phosphorous and some strontium, the primary silicon phase nucleates first along a depressed A curve, with the silicon particles having a regular shaped morphology but having a very large particle size and these silicon particles would be surrounded by a melt very low in aluminum. This subsequently causes primary aluminum dendrites to form on solidification with a eutectic forming between the dendrite arms. With no phosphorus and significant levels of strontium in the melt, the primary silicon phase is prevented from nucleating first along the A curve, but would require a greater undercooling of the melt, likely to curve C. Under these quasi-equilibrium conditions, primary aluminum may precipitate along curve C, but almost immediately massive amounts of silicon would precipitate to balance the composition imbalance. Thus, the regular shaped silicon morphology does not form as expected because of the very large undercooling of the melt and the very rapid subsequent reaction rates when a nucleation site is found in these large undercooled melts. Further, using the same chemistries in making the samples with cooling rates slower than high pressure die casting did not produce any evidence in the microstructure of the primary aluminum phase as exhibited in Fig. 8. The results of adding various amounts of strontium modifier to a chill cast 391 alloy cooling at 29°C/sec are shown in Figs. 9-10, and 12-16. Higher traditional concentrations of 0.05% Sr causes a change in the primary silicon morphology itself, resulting in a dendritic shape, as shown in Figs. 10 and 12-16.

Accordingly, 0.016% strontium is normally added to the hypoeutectic aluminum silicon alloys to modify the eutectic silicon to a fibrous morphology from an acicular morphology in the eutectic structure and to increase mechanical properties (particularly elongation). This strontium addition, however, is not expected to be effective for die cast hypereutectic Al-Si alloys because the primary silicon particle size increases by a factor of three from the 0% strontium level and machining cracks all of these silicon particles. Thus, it is unexpected to achieve smaller silicon particles with increased strontium additions in hypereutectic aluminum silicon alloys. The inventive microstructure of Fig. 8 is obtained at die casting cooling rates and cannot be obtained with permanent mold cooling rates at 0.03% strontium or at higher silicon levels near 0.20% because in these permanent mold microstructures the primary silicon is very large and dendritic [i.e., not machinable] and the eutectic is modified but the cell boundaries are decorated with small Al4Sr particles that don't precipitate at the faster cooling rates of die casting. The inventive microstructure shown in Fig. 8 includes 0.05% strontium and demonstrates refined primary silicon. Referring now to Fig. 18 therein is shown the microstructure of a similar high pressure die casting alloy but with 0.022% by weight strontium. Fig. 18 shows refined primary silicon particles and the primary aluminum phase, but also a significant number of very large primary silicon particles that are larger than the aluminum dendrite arm spacing. These large primary silicon particles have an irregular shape and likely found aluminum phosphate (AIP) or other particles to nucleate on. This is why more strontium is needed, to react with and "poison" all the conventional nuclei for primary silicon. The data suggests that the minimum strontium level to eliminate the conventional nuclei for primary silicon in the inventive hypereutectic Al-Si alloy and produce the microstructure in Figure 8 is 0.05% strontium.

The present invention is further detailed in the following example. One of skill in the art will recognize that the Aluminum Association democracy of the current listed alloys 390, 391, 392 and 393 may be modified to the inventive microstructure of Fig. 8 through the addition of 0.05 to 0.10% by weight Sr. Accordingly, the present application contemplates a hypereutectic aluminum silicon alloy comprising 16-23% by weight silicon, 0.01 to 1.5% by weight iron, 0.20 to 5.0% by weight copper, 0.01 to 0.30% by weight manganese, 0.40 to 1.3% by weight magnesium, 0.05 to 0.10% by weight strontium, and the balance aluminum wherein the alloy as cast demonstrates an algorithm of greater than 2%.

### EXAMPLE

Three "as cast" tensile specimens were extracted from engine block that was high pressure die cast with the following constituencies: 19.2% by weight Si; 0.05% by weight Sr; 0.7% by weight Fe; and 0.46% by weight Mg, with the balance aluminum, and whose microstructure is shown in Figure 8. Standard testing revealed that the alloy had average ultimate tensile strength (UTS) of 263 MPa (or 38.1 ksi), a Yield Strength of 207 MPa (or 30.0 ksi) and an elongation of 2.1%. The elongation is four times the elongation of a typical hypereutectic Al-Si alloy of 0.5%, and higher than the elongation of a well annealed conventional hypereutectic Al-Si alloy.

## Claims

1. A hypereutectic high pressure die cast aluminum silicon alloy comprising:
- 16% to 23% by weight silicon,
- 0.01% to 1.5% by weight iron,
- 0.01% to 0.6% by weight manganese,
- 0.01% to 1.3% by weight magnesium,
- 0.05% to 0.2% by weight strontium,
- optionally 0.01 % to 4.5% by weight nickel,
- optionally 0.2% to 5% copper, and
- the balance aluminum,
wherein the die cast alloy has a microstructure with a volume fraction of primary silicon of greater than 10%.

2. The hypereutectic aluminum silicon alloy of claim 1, **characterized in that** the alloy has a microstructure with a volume fraction of primary silicon at 10% to 20%, a volume fraction of modified aluminum-silicon eutectic at 45% to 90%, and the balance of the microstructure primary aluminum.

3. The hypereutectic aluminum silicon alloy of claim 1 or 2, **characterized in that** the volume fraction of primary silicon is surrounded by divorced eutectic aluminum.

4. The hypereutectic aluminum silicon alloy according to claim 3, **characterized in that** the volume fracture of primary aluminum, including the divorced eutectic aluminum surrounding the primary aluminum is larger than the volume fraction of primary silicon.

5. The hypereutectic aluminum silicon alloy according to claim 2, **characterized in that** the volume fraction of modified aluminum-silicon eutectic includes fibrous eutectic silicon.

6. The hypereutectic aluminum silicon alloy according to any one of the preceding claims, **characterized in that** the microstructure primary aluminum is dendritic with an average dendritic arm spacing of less than 15 µm.

7. The hypereutectic aluminum silicon alloy according to claim 6, **characterized in that** the primary aluminum dendritic arm spacing is larger than the average primary silicon particle size.

8. The hypereutectic aluminum silicon alloy according to any one of the preceding claims, **characterized in that** it comprises 0.01% to 0.7%, preferably 0.01% to 0.2%, by weight iron.

9. The hypereutectic aluminum silicon alloy according to any one of the preceding claims, **characterized in that** it comprises 0.01% to 0.5% by weight manganese.

10. The hypereutectic aluminum silicon alloy according to any one of the preceding claims, **characterized in that** it comprises 0.05% to 0.1% by weight strontium.

11. The hypereutectic aluminum silicon alloy according to any one of the preceding claims, **characterized in that** it has an average ultimate tensile strength of greater than 250 MPa.

12. The hypereutectic aluminum silicon alloy according to any one of the preceding claims, **characterized in that** it has a yield strength of greater than 200 MPa.

13. The hypereutectic aluminum silicon alloy according to any one of the preceding claims, **characterized in that** the alloy microstructure exhibits an elongation of at least 2%.

14. The hypereutectic aluminum silicon alloy according to any one of the preceding claims, **characterized in that** the average primary silicon particle size is less than 10 µm.

15. The hypereutectic aluminum silicon alloy according to claim 1, **characterized in that** it comprises 0.01 to 0.3% by weight manganese, 0.4 to 1.3% by weight magnesium and 0.05 to 0.1% by weight strontium, and that it further comprises 0.2% to 5% by weight copper, and that the alloy when cast demonstrates an elongation of greater than 2%.

## Patentansprüche

1. Hypereutektische Aluminium-Silizium-Hochdruckgusslegierung, umfassend:
- 16 bis 23 Gewichtsprozent Silizium,
- 0,01 bis 1,5 Gewichtsprozent Eisen,
- 0,01 bis 0,6 Gewichtsprozent Mangan,
- 0,01 bis 1,3 Gewichtsprozent Magnesium,
- 0,05% bis 0,2% Gewichtsprozent Strontium,
- optional 0,01 bis 4,5 Gewichtsprozent Nickel,
- wahlweise 0,2 % bis 5 % Kupfer, und
- restlicher Anteil Aluminium,
wobei die Druckgusslegierung eine Mikrostruktur mit einem Volumenanteil von Primärsilizium von mehr als 10 % aufweist.

2. Hypereutektische Aluminium-Silizium-Legierung nach Anspruch 1, **dadurch gekennzeichnet, dass**
die Legierung eine Mikrostruktur mit einem Volumenanteil von Primärsilizium von 10 % bis 20 %, einem Volumenanteil von modifiziertem Aluminium-Silizium-Eutektikum von 45 % bis 90 % und dem restlichen Anteil der Mikrostruktur von Primäraluminium aufweist.

3. Hypereutektische Aluminium-Silizium-Legierung nach Anspruch 1 oder 2, **dadurch gekennzeichnet, dass** der Volumenanteil von Primärsilizium von abgetrenntem eutektischem Aluminium umgeben ist.

4. Hypereutektische Aluminium-Silizium-Legierung nach Anspruch 3, **dadurch gekennzeichnet, dass** der Volumenanteil von Primäraluminium, einschließlich des abgetrennten eutektischen Aluminiums, das das Primäraluminium umgibt, größer ist als der Volumenanteil von Primärsilizium.

5. Hypereutektische Aluminium-Silizium-Legierung nach Anspruch 2, **dadurch gekennzeichnet, dass** der Volumenanteil von modifiziertem Aluminium-Silizium-Eutektikum faserförmiges eutektisches Silizium enthält.

6. Hypereutektische Aluminium-Silizium-Legierung nach einem der vorhergehenden Ansprüche, **dadurch gekennzeichnet, dass** das Primäraluminium in der Mikrostruktur dendritisch ist mit einem durchschnittlichen Abstand der Dendritenarme von weniger als 15 µm.

7. Hypereutektische Aluminium-Silizium-Legierung nach Anspruch 6, **dadurch gekennzeichnet, dass** der Abstand der Primäraluminium-Dendritenarme größer ist als die durchschnittliche Partikelgröße des Primärsiliziums.

8. Hypereutektische Aluminium-Silizium-Legierung nach einem der vorhergehenden Ansprüche, **dadurch gekennzeichnet, dass** sie 0,01 bis 0,7 Gewichtsprozent, vorzugsweise 0,01 bis 0,2 Gewichtsprozent, Eisen enthält.

9. Hypereutektische Aluminium-Silizium-Legierung nach einem der vorhergehenden Ansprüche, **dadurch gekennzeichnet, dass** sie 0,01 bis 0,5 Gewichtsprozent Mangan enthält.

10. Hypereutektische Aluminium-Silizium-Legierung nach einem der vorhergehenden Ansprüche, **dadurch gekennzeichnet, dass** sie 0,05 bis 0,1 Gewichtsprozent Strontium enthält.

11. Hypereutektische Aluminium-Silizium-Legierung nach einem der vorhergehenden Ansprüche, **dadurch gekennzeichnet, dass** sie eine mittlere Zugfestigkeit von mehr als 250 MPa aufweist.

12. Hypereutektische Aluminium-Silizium-Legierung nach einem der vorhergehenden Ansprüche, **dadurch gekennzeichnet, dass** sie eine Streckgrenze von mehr als 200 MPa aufweist.

13. Hypereutektische Aluminium-Silizium-Legierung nach einem der vorhergehenden Ansprüche, **dadurch gekennzeichnet, dass** die Legierungsmikrostruktur eine Dehnung von mindestens 2% zeigt.

14. Hypereutektische Aluminium-Silizium-Legierung nach einem der vorhergehenden Ansprüche, **dadurch gekennzeichnet, dass** die durchschnittliche Partikelgröße des Primärsiliziums weniger als 10 µm beträgt.

15. Hypereutektische Aluminium-Silizium-Legierung nach Anspruch 1, **dadurch gekennzeichnet, dass** sie 0,01 bis 0,3 Gewichtsprozent Mangan, 0,4 bis 1,3 Gewichtsprozent Magnesium und 0,05 bis 0,1 Gewichtsprozent Strontium enthält, und dass sie ferner 0,2 bis 5 Gewichtsprozent Kupfer enthält, und dass die Legierung beim Gießen eine Dehnung von mehr als 2 % zeigt.

## Revendications

1. Alliage hypereutectique d'aluminium-silicium coulé sous haute pression comprenant :
- 16% à 23% en poids de silicium,
- 0,01% à 1,5% en poids de fer,
- 0,01% à 0,6% en poids de manganèse,
- 0,01% à 1,3% en poids de magnésium,
- 0,05% à 0,2% en poids de strontium,
- optionnel 0,01% à 4,5% en poids de nickel,
- optionnel 0,2 % à 5 % de cuivre, et
- parts restante d'aluminium,
dans lequel l'alliage coulé sous pression a une microstructure avec une fraction volumique de silicium primaire supérieure à 10 %.

2. Alliage hypereutectique d'aluminium-silicium selon la revendication 1, **caractérisé en ce que**
l'alliage a une microstructure avec une fraction volumique de silicium primaire de 10 % à 20 %, une fraction volumique d'eutectique aluminium-silicium modifié de 45 % à 90 %, et le reste de la microstructure en aluminium primaire.

3. Alliage hypereutectique d'aluminium-silicium selon la revendication 1 ou 2, **caractérisé en ce que** la fraction volumique de silicium primaire est entourée d'aluminium eutectique divorcé.

4. Alliage hypereutectique d'aluminium-silicium selon la revendication 3, **caractérisé en ce que** la fraction volumique de l'aluminium primaire, y compris l'aluminium eutectique divorcé entourant l'aluminium primaire, est supérieure à la fraction volumique du silicium primaire.

5. Alliage hypereutectique d'aluminium-silicium selon la revendication 2, **caractérisé en ce que** la fraction volumique de l'eutectique aluminium-silicium modifié comprend du silicium eutectique fibreux.

6. Alliage hypereutectique d'aluminium-silicium selon l'une quelconque des revendications précédentes, **caractérisé en ce que** la microstructure de l'aluminium primaire est dendritique avec un espacement moyen des bras dendritiques inférieur à 15 µm.

7. Alliage hypereutectique d'aluminium-silicium selon la revendication 6, **caractérisé en ce que** l'espacement des bras dendritiques d'aluminium primaire est plus grand que la taille moyenne des particules de silicium primaire.

8. Alliage hypereutectique d'aluminium-silicium selon l'une quelconque des revendications précédentes, **caractérisé en ce qu'**il comprend 0,01% à 0,7%, de préférence 0,01% à 0,2%, en poids de fer.

9. Alliage hypereutectique d'aluminium-silicium selon l'une quelconque des revendications précédentes, **caractérisé en ce qu'**il comprend 0,01% à 0,5% en poids de manganèse.

10. Alliage hypereutectique d'aluminium-silicium selon l'une quelconque des revendications précédentes, **caractérisé en ce qu'**il comprend 0,05% à 0,1% en poids de strontium.

11. Alliage hypereutectique d'aluminium-silicium selon l'une quelconque des revendications précédentes, **caractérisé en ce qu'**il présente une résistance moyenne à la rupture supérieure à 250 MPa.

12. Alliage hypereutectique d'aluminium-silicium selon l'une quelconque des revendications précédentes, **caractérisé en ce qu'**il présente une limite élastique supérieure à 200 MPa.

13. Alliage hypereutectique d'aluminium-silicium selon l'une quelconque des revendications précédentes, **caractérisé en ce que** la microstructure de l'alliage présente une élongation d'au moins 2%.

14. Alliage hypereutectique d'aluminium-silicium selon l'une quelconque des revendications précédentes, **caractérisé en ce que** la taille moyenne des particules de silicium primaire est inférieure à 10 µm.

15. Alliage hypereutectique d'aluminium-silicium selon la revendication 1, **caractérisé en ce qu'**il comprend 0,01 à 0,3 % en poids de manganèse, 0,4 à 1,3 % en poids de magnésium et 0,05 à 0,1 % en poids de strontium, et **en ce qu'**il comprend en outre 0,2 % à 5 % en poids de cuivre, et **en ce que** l'alliage, lorsqu'il est coulé, présente une élongation supérieur à 2 %.
